



US010113270B2

(12) **United States Patent**  
**Gray et al.**

(10) **Patent No.:** **US 10,113,270 B2**  
(b4) **Date of Patent:** **Oct. 30, 2018**

(54) **PROCESS FOR THE MANUFACTURE OF PAPER AND PAPERBOARD**

(71) Applicant: **BASF SE**, Ludwigshafen (DE)

(72) Inventors: **Christopher Alan Gray**, Limburgerhof (DE); **Antonius Moormann-Schmitz**, Gruenstadt (DE); **Hubert Meixner**, Ludwigshafen (DE); **Luis Miguel Sanchez Cerro**, Heidelberg (DE); **Thomas Muehlenbernd**, Heidelberg (DE); **Christian Jahn-Rendu**, Pudong New Area (CN)

(73) Assignee: **BASF SE**, Ludwigshafen (DE)

(\*) Notice: Subject to any disclaimer, the term of this patent is extended or adjusted under 35 U.S.C. 154(b) by 0 days.

(21) Appl. No.: **14/760,381**

(22) PCT Filed: **Jan. 9, 2014**

(86) PCT No.: **PCT/IB2014/058145**

§ 371 (c)(1),  
(2) Date: **Jul. 10, 2015**

(87) PCT Pub. No.: **WO2014/108844**

PCT Pub. Date: **Jul. 17, 2014**

(65) **Prior Publication Data**

US 2015/0345081 A1 Dec. 3, 2015

(30) **Foreign Application Priority Data**

Jan. 11, 2013 (WO) ..... PCT/CN2013/070355

(51) **Int. Cl.**

**D21H 17/44** (2006.01)  
**D21H 17/68** (2006.01)  
**D21H 21/18** (2006.01)  
**D21H 17/56** (2006.01)  
**D21H 21/10** (2006.01)  
**D21H 17/37** (2006.01)  
**D21H 17/00** (2006.01)  
**D21H 11/20** (2006.01)  
**D21H 17/45** (2006.01)  
**D21H 17/55** (2006.01)  
**D21H 23/04** (2006.01)  
**D21H 23/18** (2006.01)

(52) **U.S. Cl.**

CPC ..... **D21H 17/74** (2013.01); **D21H 11/20** (2013.01); **D21H 17/375** (2013.01); **D21H 17/44** (2013.01); **D21H 17/45** (2013.01); **D21H 17/55** (2013.01); **D21H 17/68** (2013.01); **D21H 21/10** (2013.01); **D21H 23/04** (2013.01); **D21H 23/18** (2013.01)

(58) **Field of Classification Search**

CPC ..... D21H 21/10; D21H 17/455; D21H 23/14; D21H 17/375; D21H 17/37; D21H 17/56; D21H 17/68; D21H 17/44; D21H 17/55; D21H 17/45; D21H 17/74; D21H 17/36; D21H 17/67; D21H 17/63; D21H 23/26; D21H 27/30

See application file for complete search history.

(56) **References Cited**

U.S. PATENT DOCUMENTS

|             |         |                           |
|-------------|---------|---------------------------|
| 4,388,150 A | 6/1983  | Sunden et al.             |
| 4,421,602 A | 12/1983 | Brannmueller et al.       |
| 5,482,693 A | 1/1996  | Rushmere et al.           |
| 5,536,370 A | 7/1996  | Scherr et al.             |
| 5,641,855 A | 6/1997  | Scherr et al.             |
| 5,676,796 A | 10/1997 | Cutts                     |
| 6,056,967 A | 5/2000  | Steuerle et al.           |
| 6,103,065 A | 8/2000  | Humphreys et al.          |
| 6,132,558 A | 10/2000 | Dyllick-Brenzinger et al. |

(Continued)

FOREIGN PATENT DOCUMENTS

|    |              |        |       |             |
|----|--------------|--------|-------|-------------|
| CA | 2180373 A1 * | 8/1997 | ..... | D21H 23/765 |
| CA | 2354106 A1 * | 8/1997 | ..... | D21H 23/765 |

(Continued)

OTHER PUBLICATIONS

International Search Report issued May 8, 2014 in PCT/IB2014/058145.

International Preliminary Report on Patentability and Written Opinion issued Jul. 23, 2015 in PCT/IB2014/058145.

Ying Huang, et al., "Synthesis and characterization of bisacrylamide microgels containing sulfo groups" Makromol. Chem., vol. 186, 1985, pp. 273-281.

Office Action dated Oct. 3, 2016 in corresponding Japanese Patent Application No. 2015-552177—English Translation Only.

(Continued)

Primary Examiner — Jose A Fortuna

(74) Attorney, Agent, or Firm — Oblon, McClelland, Maier & Neustadt, L.L.P.

(57) **ABSTRACT**

Process for the Manufacture of Paper and Paperboard The present invention relates to a process of making paper or paperboard in which a cellulosic thin stock is provided and subjected to one or more shear stages and then drained and a moving screen to form a sheet which is dried, wherein the process employs a retention system which is applied to the thin stock, said retention system comprising as components i) a blend of different cationic polymers and ii) a microparticulate material, in which the blend of cationic polymers comprises, a) a cationic polymer having a charge density of from 0.5 and below 3 mEq per gram and a molar mass of greater than 700,000 Da, which cationic polymer is selected from polymers containing vinyl amine units and polyethyl-enimine, b) a cationic polymer having a charge density of below 3 mEq per gram and an intrinsic viscosity of at least 3 dl/g, wherein one of the components of the retention system is dosed into the thin stock after the final shearing stage and the other is dosed into the thin stock before the final shearing stage.

| (56)                     | References Cited |                    |             |                                                                                                                         |         |            |
|--------------------------|------------------|--------------------|-------------|-------------------------------------------------------------------------------------------------------------------------|---------|------------|
| U.S. PATENT DOCUMENTS    |                  |                    |             |                                                                                                                         |         |            |
| 6,706,190 B1             | 3/2004           | Steuerle et al.    | EP          | 0 235 893 A1                                                                                                            | 9/1987  |            |
| 7,306,701 B2             | 12/2007          | Blum et al.        | EP          | 0 335 575 A2                                                                                                            | 10/1989 |            |
| 7,388,025 B2             | 6/2008           | Buettelmann et al. | EP          | 0 484 617 A1                                                                                                            | 5/1992  |            |
| 7,795,340 B2             | 9/2010           | Wester et al.      | EP          | 0 485 124 A1                                                                                                            | 5/1992  |            |
| 7,998,314 B2             | 8/2011           | Koch et al.        | EP          | 0 752 496 A2                                                                                                            | 1/1997  |            |
| 8,454,796 B2 *           | 6/2013           | Reinicke .....     | D21H 21/10  | 0 877 120                                                                                                               | 11/1998 |            |
|                          |                  |                    | 162/164.6   | 1 945 683                                                                                                               | 4/1999  |            |
| 9,103,071 B2             | 8/2015           | Jehn-Rendu         | EP          | 1 948 648 A                                                                                                             | 7/2008  |            |
| 9,404,223 B2 *           | 8/2016           | Gray .....         | D21H 17/375 | 1 509 967 A                                                                                                             | 7/2008  |            |
| 9,631,319 B2 *           | 4/2017           | Gray .....         | D21H 17/74  | JP H06-509851                                                                                                           | 5/1978  |            |
| 2005/0247420 A1 *        | 11/2005          | Blum .....         | D21H 23/18  | 2000-514144                                                                                                             | 11/1994 |            |
|                          |                  |                    | 162/158     | JP 2005-054311                                                                                                          | 10/2000 |            |
| 2007/0105922 A1          | 5/2007           | Buettelmann et al. | JP          | 2005-534824                                                                                                             | 3/2005  |            |
| 2008/0000601 A1          | 1/2008           | Leduc et al.       | JP          | 2008-525668                                                                                                             | 11/2005 |            |
| 2008/0287596 A1          | 11/2008          | Wester et al.      | JP          | WO 86/00100 A1                                                                                                          | 7/2008  |            |
| 2010/0089541 A1 *        | 4/2010           | Reinicke .....     | D21H 21/10  | WO 9325754                                                                                                              | 1/1986  |            |
|                          |                  |                    | 162/164.6   | WO 94/12560 A1                                                                                                          | 12/1993 |            |
| 2010/0282424 A1          | 11/2010          | Koch et al.        | WO          | WO 94/14873 A1                                                                                                          | 6/1994  |            |
| 2014/0367059 A1 *        | 12/2014          | Gray .....         | D21H 17/375 | WO 97/23567 A1                                                                                                          | 7/1994  |            |
|                          |                  |                    | 162/127     | WO 97/25367 A1                                                                                                          | 7/1997  |            |
| 2015/0027650 A1 *        | 1/2015           | Gray .....         | D21H 17/44  | WO 97/33040 A1                                                                                                          | 9/1997  |            |
|                          |                  |                    | 162/164.2   | WO 97/33041 A1                                                                                                          | 9/1997  |            |
| 2015/0345081 A1 *        | 12/2015          | Gray .....         | D21H 17/45  | WO 98/01623 A1                                                                                                          | 5/1998  |            |
|                          |                  |                    | 162/168.3   | WO 98/22653                                                                                                             | 1/1998  |            |
|                          |                  |                    |             | WO 99/16708 A1                                                                                                          | 4/1999  |            |
|                          |                  |                    |             | WO 00/67884 A1                                                                                                          | 5/1999  |            |
|                          |                  |                    |             | WO 2006071961 A1 *                                                                                                      | 11/2000 |            |
|                          |                  |                    |             | WO 2006071961 A1 *                                                                                                      | 7/2006  | D21H 21/10 |
|                          |                  |                    |             | WO 2007/051736 A1                                                                                                       | 5/2007  |            |
|                          |                  |                    |             | WO 2007/054444 A2                                                                                                       | 5/2007  |            |
|                          |                  |                    |             | WO 2014108844 A1 *                                                                                                      | 7/2014  | D21H 17/45 |
| FOREIGN PATENT DOCUMENTS |                  |                    |             |                                                                                                                         |         |            |
| CA 2862095 C *           | 4/2017           |                    | D21H 17/375 | OTHER PUBLICATIONS                                                                                                      |         |            |
| CN WO 2014108844 A1 *    | 7/2014           |                    | D21H 17/45  | Extended European Search Report dated Jun. 30, 2016, in European Patent Application No. 14738178.4, filed Jan. 9, 2016. |         |            |
| DE 24 34 816 A1          | 2/1976           |                    |             | *                                                                                                                       |         |            |
| DE 102 36 252            | 5/2003           |                    |             | cited by examiner                                                                                                       |         |            |
| EP 0 071 050 A1          | 2/1983           |                    |             |                                                                                                                         |         |            |
| EP 0 102 760 A2          | 3/1984           |                    |             |                                                                                                                         |         |            |
| EP 0 126 528 A2          | 11/1984          |                    |             |                                                                                                                         |         |            |
| EP 0 150 933 A2          | 8/1985           |                    |             |                                                                                                                         |         |            |

## 1

PROCESS FOR THE MANUFACTURE OF  
PAPER AND PAPERBOARD

The present invention relates to a method for the manufacture of paper and paperboard from a cellulosic suspension, employing a novel retention system.

## BACKGROUND OF THE INVENTION

It is well known to manufacture paper by a process that comprises flocculating a cellulosic thin stock by the addition of polymeric retention aid and then draining the flocculated suspension through a moving screen (often referred to as a machine wire) and then forming a wet sheet, which is then dried.

In order to increase output of paper many modern paper making machines operate at higher speeds. As a consequence of increased machine speeds a great deal of emphasis has been placed on drainage and retention systems that provide increased drainage. However, it is known that increasing the molecular weight of a polymeric retention aid which is added immediately prior to drainage will tend to increase the rate of drainage but damage formation. It is difficult to obtain the optimum balance of retention, drainage, drying and formation by adding a single polymeric retention aid and it is therefore common practice to add two separate materials in sequence.

EP-A-235893 provides a process wherein a water soluble substantially linear cationic polymer is applied to the paper making stock prior to a shear stage and then reflocculating by introducing bentonite after that shear stage. This process provides enhanced drainage and also good formation and retention. This process which is commercialized by BASF under the Hydrocol® (trade mark) has proved successful for more than two decades.

This Hydrocol® (trade mark) system of making paper is a very efficient microparticle system for a wide range of paper grades including liner board and folding box board production. The benefits of this system include high retention levels, good drainage, good formation, good machine cleanliness, good runnability and a cost efficient system.

Subsequently, various attempts have been made to provide variations on this theme by making minor modifications to one or more of the components.

EP-A-335575 describes such a process in which a main polymer selected from cationic starch and high molecular weight water-soluble cationic polymer is added to a cellulosic suspension after which the suspension is passed through one or more shear stages followed by the addition of inorganic material selected from bentonite and colloidal silica. In this system a low molecular weight cationic polymer is added into the suspension before the addition of the main polymer. It is indicated that the low molecular weight polymer usually has a molecular weight below 500,000 and usually above 50,000, often above 100,000. Suggested low molecular weight cationic polymers include polyethyleneimine, polyamines, polymers of dicyandiamidesformaldehyde, polymers and copolymers of diallyl dimethyl ammonium chloride, of dialkyl amino alkyl(meth)acrylates and of dialkyl amino alkyl(meth)acrylamides (both generally as acid addition or quaternary ammonium salts). The process was said to improve processes in which there is a high amount of pitch or processes with a high cationic demand.

A further development of this type of process was subsequently disclosed in EP-A-910701 in which two different water-soluble cationic polymers are added in succession to

## 2

pulps followed by subjecting the pulps to at least one shearing stage followed by the addition of bentonite, colloidal silica or clay. Specifically polyethyleneimines having a molar mass of more than 500,000 or polymers containing vinyl amine groups having a molar mass of between 5000 and 3 million are added to the pulp and then high molecular weight cationic polyacrylamides.

EP-A-752496 discloses a papermaking process in which a low molecular weight cationic polymer having a molecular weight below 700,000 and a cationic and/or amphoteric high molecular weight polymer are added simultaneously to the thin stock with anionic inorganic particles such as silica or bentonite being dosed into the thin stock suspension. The low molecular weight cationic polymer includes polyethyleneimine and polyvinyl amine. The polymers are generally added separately although it is indicated that the two cationic polymers can be added as a mixture. It is also indicated that the polymers can be added before a shear stage although the exact addition points are not indicated. It is stated that this process results in improved drainage and/or retention compare to processes in which the high molecular weight cationic or amphoteric polymer is used alone in conjunction with anionic inorganic particles.

U.S. Pat. No. 6,103,065 discloses a papermaking process involving the addition to a paper stock after the last point of high shear at least one high charge density cationic polymer of molecular weight between 100,000 and 2 million with a charge density in excess of 4 mEq per gram and either concurrently or subsequently adding at least one polymer having a molecular weight more than 2 million with a charge density below 4 mEq per gram. Subsequent to the two polymers a swellable bentonite clay is added to the stock. The high charge density polymer can be polyethyleneimine homopolymers or copolymers or polymers produced from vinyl amines. This document indicates that the process improves conventional bentonite programs by employing less polymer and improving press section dewatering which increases the solids entering the dryers thereby reducing the drying requirements.

In the production of paper and paperboard the paper machine can become limited by the amount of water retained in the final web after the press section when the paper machine is using maximum drying energy. The retention of fibre and filler articles is also limited when using standard retention and drainage aid systems due to potential paper quality issues. The retention and dewatering performance can be improved by using higher additions of retention and drainage aid chemicals such as polyacrylamide and bentonite. However, larger doses of these chemicals can negatively impact on the physical properties of the paper sheet.

A particular disadvantage of many conventional microparticle systems is that drainage tends to increase simultaneously with increasing retention. Although this may have been perceived as an advantage several years ago, with modern high-speed paper machines very high drainage can be a disadvantage. This can be the case for gap former machines and multi-ply fourdrinier machines. Folding box board is normally produced on multi-ply fourdrinier machines in which the major ply is the middle layer (typically about 150 to 400 g/m<sup>2</sup>). The requirements for these grades are good retention for the lower basis weight and good drainage for the high basis weight. Nevertheless in most cases it is necessary to reduce the paper machine speed for the higher basis weight sheets because of these drainage limitations. In many cases simply increasing the retention aid components the drainage on the wire can be improved

but the water release in the press tends to be reduced. Further, formation can also be adversely affected.

It would be desirable to provide an improved process for making paper and board. Furthermore, it would be desirable to overcome the aforementioned disadvantages.

#### BRIEF SUMMARY OF THE INVENTION

According to the present invention we provide a process of making paper or paperboard in which a cellulosic thin stock is provided and subjected to one or more shear stages and then drained and a moving screen to form a sheet which is dried, wherein the process employs a retention system which is applied to the thin stock, said retention system comprising as components,

- i) a blend of different cationic polymers and
  - ii) a microparticulate material,
- in which the blend of cationic polymers comprises,
- a) a cationic polymer having a charge density of from 0.5 and below 3 mEq per gram and a molar mass of greater than 700,000 Da, which cationic polymer is selected from polymers containing vinyl amine units and polyethylenimine,
  - b) a cationic polymer having a charge density of below 3 mEq per gram and an intrinsic viscosity of at least 3 dl/g,

wherein one of the components of the retention system is dosed into the thin stock after the final shearing stage and the other is dosed into the thin stock before the final shearing stage.

The inventors found that the process of the present invention conveniently allows for the machines speed to be increased, especially when making board, such as folding box board. Additionally, the process allows improved retention without necessarily increasing drainage. Such an improvement may be regarded as a decoupling effect between retention and drainage. Further, the process appears to allow runnability. The sheets of paper and board produced by the process of the present invention also exhibit improved formation and strength. Furthermore, this process allows increased productivity of the paper and board.

#### DETAILED DESCRIPTION OF THE INVENTION

In the process of making paper or paperboard a cellulosic thin stock is typically made by first forming a thick stock suspension from stock material and water and then diluting this thick stock suspension with dilution water to form the cellulosic thin stock. The thin stock will be passed through one or more shear stages and then drained on a moving screen (often termed machine wire) to form a wet sheet which can then be dried. In the case of making paperboard several layers or plies may be combined to form a composite sheet. Typically, a thin stock suspension may have a stock consistency of between 0.1 and 3% solids on total weight of suspension.

In a process of making paper or paperboard there may be several shearing stages, selected from mixing, pumping and screening. Usual shearing stages include the one or more fan pumps or the one or more pressure screens. Typically the final shearing stage is often a pressure screen. Following this final shearing stage the thin stock may typically be fed into a headbox or constant flow box which delivers the thin stock onto the moving screen often termed machine wire.

The paper may be formed as single ply sheets. However, the process is particularly suitable for making multiple layer

or multi-ply sheets, particularly in the case of board manufacture. The base weight of the respective layers may be the same, similar or different. In some cases, such as in the manufacture of folding box board it is the middle layer which has a higher base weight, for instance between 150 and 400 g/m<sup>2</sup>. The process of the present invention is particularly suitable for the manufacture of board.

According to the process of the present invention multiply least one of the retention components can be added after the final shearing stage whilst the other should be added before this point. It may be desirable to add the first retention component to the thin stock and then pass the so treated thin stock through more than one shear stage and then after the last shearing stage to add the other retention component.

It may be desirable in some cases to dose the microparticle material to the thin stock before the last shearing stage and then subsequent to this stage dosing the blend of cationic polymers. Nevertheless, it is preferred that the blend of cationic polymers is dosed into the thin stock before the final shearing stage and then the microparticle material dosed into the thin stock after the final shearing stage.

The cationic polymer (a) of the blend which has a charge density of from 0.5 to below 3 mEq per gram may be any one of a number of types of cationic polymers provided that it has a molar mass greater than 700,000 Da. The molar mass may be as high as 3,000,000 Da but is generally up to 2,000,000 Da or 2,500,000 Da. Suitably the molar mass may be at least 750,000 Da and often at least 800,000 Da. Often the molar mass will be at least 900,000 Da or even at least 1,000,000 Da or in some cases at least 1,100,000 Da or even at least 1,500,000 Da. The molar mass may for instance be between 1,000,000 Da and 2,000,000 Da or 2,500,000 Da or 3,000,000 Da, for instance 1,100,000 Da to 1,800,000 Da. A preferred molar mass is from 1.5 to 2.5 million Da. The charge density may be at least 1 mEq per gram or at least 1.5 mEq per gram. The charge density may for instance be any value higher than this for instance up to 2.0 or 2.5 or 2.7 mEq per gram provided that it is below 3 mEq per gram. Suitably this cationic polymer may be any of the polymers generally described as polyethylenimines, modified polyethylenimines, polymers of vinyl carboxamides, such as N-vinyl formamide, followed by partial or complete hydrolysis to yield vinyl amine units. Preferred polymers are selected from the group consisting of polyvinylamines, and partially hydrolysed polyvinyl carboxamides.

Especially preferred cationic polymers of component (a) include polyvinyl amines (including any polymer having vinyl amine units) with a charge density from 1 to 2 mEq per gram and having a molar mass of from 1.5 to 2.5 million Da.

The molar mass can be determined for example by static light scattering, small angle neutron scattering, x-ray scattering or sedimentation velocity.

Charge density of the cationic polymers can be determined by titration of an aqueous solution of the polymer with potassium polyvinyl sulphate (KPVS). A suitable indicator can be used, for instance o-toluidine blue.

Charge density (LA), measured in milliequivalents per gram, can be determined as follows:

$$LA = \frac{KV \times CK \times FK}{PT}$$

Where

FK is the correction factor for the nonvolatile fraction of the polymer solution.

$$FK = TN/FR$$

TN is the theoretical nonvolatile fraction of the polymer solution;

FR is the measured nonvolatile fraction of the polymer solution;

KV is the volume of KPVS used in the titration, in ml;

CK is the concentration of KPVS solution, in milliequivalents/ml;

PT is the theoretical mass of the polymer used, in grams.

Polyethyleneimines or modified polyethyleneimines may be as defined below include the nitrogen-containing condensation products described in German laid-open specification DE 24 34 816. These are obtained by reacting polyamidoamine compounds with polyalkylene oxide derivatives whose terminal hydroxyl groups have been reacted with epichlorohydrin. Other suitable polyethyleneimines are described in WO 97/25367 A1, WO 94/14873 A1, and WO 94/12560 A1. The polyethyleneimines or modified polyethyleneimines may be subsequently subjected to ultrafiltration as described in WO 00/67884 A1 and WO 97/23567 A1. Suitable polyethyleneimines and modified polyethyleneimines include polyalkylenimines, polyalkylene polyamines, polyamidoamines, polyalkylene glycol polyamines, polyamidoamines grafted with ethylenimine and subsequently reacted with at least difunctional crosslinkers, and mixtures and copolymers thereof.

The preferred cationic polymers (a) having a charge density of from 0.5 to below 3 mEq per gram and a molar mass greater than 700,000 Da polymers containing vinyl amine units. These include partially hydrolysed polyvinyl carboxamides. More preferably these cationic polymers are homopolymers or copolymers of N-vinylformamide. These may be obtained by polymerizing N-vinylformamide to give homopolymers or by copolymerizing N-vinylformamide together with at least one other ethylenically unsaturated monomer. The vinylformamide units of these polymers are not hydrolyzed, in contradistinction to the preparation of polymers comprising vinylamine units. The copolymers may be cationic, anionic or amphoteric. Cationic polymers are obtained, for example, by copolymerizing N-vinylformamide with at least one other compatible ethylenically unsaturated water-soluble monomer, for instance acrylamide. Such polymers may for instance be produced as in aqueous solution, as a powder, as a reverse-phase emulsion or dispersion or as an aqueous dispersion.

Polymers comprising vinylformamide units are known. For instance, EP-A 0 071 050 describes linear basic polymers comprising 90 to 10 mol % of vinylamine units and 10 to 90 mol % of vinylformamide units. These polymers are produced by polymerizing N-vinylformamide by the solution polymerization process in water, the inverse suspension polymerization process, the water-in-oil emulsion polymerization process or the precipitation polymerization process and, in each case, subsequent partial detachment of formyl groups from the polyvinylformamides to form vinylamine units.

It is also suitable to produce a polymer powder comprising vinylformamide units by free radical polymerization of an aqueous solution of N-vinylformamide and if appropriate other monomers and drying the polymer. Typically this comprises an aqueous monomer solution comprising N-vinylformamide and at least one polymerization initiator being spray dispensed as an aerosol or dropletized at the top of a

heatable tower-shaped reactor. Then the aerosol or droplets are polymerised in an inert gas atmosphere to form a finely divided solid followed by discharging the finely divided polymer from the reactor. This is for instance described in EP 1948648.

Another particularly desirable form of such poly vinyl carboxamides includes aqueous dispersions. Such aqueous dispersions of water-soluble polymers of N-vinylcarboxamides, may be characterised in being substantially salt-free and comprising anionic polymeric stabilizers having a comb-like molecular structure. The aqueous dispersions may contain at least one polymeric stabilizer having a comb-like molecular structure, which is obtained by copolymerization of monomer mixtures comprising macromonomers and which is present as an anion under the polymerization conditions. The structure of the stabilizers can be described, for example, as a hydrocarbon backbone with anionic groups and nonpolar polyalkylene glycol side chains. In the aqueous polymerization medium, these stabilizers act, for example, as a stabilizer and/or as a precipitating agent for the polymer particles forming. These polymers may be obtained by copolymerization of monomer mixtures comprising macromonomers, for example as described in EP 1945683.

Mixtures of from 25 or 50 to 100% by weight of N-vinylformamide and from 0 to 50 or 75% by weight of one or more of said comonomers are suitable for the preparation of the water-soluble N-vinylcarboxamide polymers. The aqueous dispersions may be substantially salt-free. Here, "substantially salt-free" means that any amount of inorganic salts which is still present in the dispersions is very small, preferably less than about 1% by weight, particularly preferably less than 0.5% by weight and very particularly preferably less than 0.3% by weight in total, based in each case on the total weight of the aqueous dispersion. The aqueous dispersions of watersoluble polymers of N-vinylcarboxamides preferably have a high polymer content and preferably comprise polymers having high molar masses and simultaneously a low viscosity.

The cationic polymer (b) having a charge density of below 3 mEq per gram and an intrinsic viscosity of at least 4 dl/g desirably may be prepared using a water-soluble ethylenically unsaturated monomer or blend of water-soluble ethylenically unsaturated monomers in which at least one of the monomers is cationic. Where the polymers are formed from more than one monomer the other monomers may be either cationic or non-ionic or a mixture, although it may be desirable for said monomers to include one or more anionic monomers resulting in an amphoteric polymer, provided that the overall charge is cationic. Nevertheless it is preferred that the two polymeric retention aids are formed entirely from cationic monomer or a mixture of monomers containing at least one cationic monomer and at least one non-ionic monomer.

The cationic monomers include dialkylamino alkyl(meth) acrylates, dialkylamino alkyl(meth)acrylamides, including acid addition and quaternary ammonium salts thereof, diallyl dimethyl ammonium chloride. Preferred cationic monomers include the methyl chloride quaternary ammonium salts of dimethylamino ethyl acrylate and dimethyl aminoethyl methacrylate. Suitable non-ionic monomers include unsaturated nonionic monomers, for instance acrylamide, methacrylamide, hydroxyethyl acrylate, N-vinylpyrrolidone. A particularly preferred polymer includes the copolymer of acrylamide with the methyl chloride quaternary ammonium salts of dimethylamino ethyl acrylate.

This cationic polymer preferably contains at least 5 mol % cationic monomer units and up to 60 mol % cationic monomer units, more preferably between 5 and 40 mol % cationic monomer units, especially between 5 and 20 mol %. A particularly preferred first polymeric retention aids are also cationic polyacrylamides comprising acrylamide and at least one water-soluble cationic ethylenically unsaturated monomer, preferably quaternary ammonium salts of dialkyl amino alkyl(meth)-acrylates or N-substituted-acrylamides, especially the methyl chloride quaternary ammonium salts of dimethylamino ethyl acrylate.

Preferably the first polymeric retention aid exhibits an intrinsic viscosity of at least 5 and often at least 6 dl/g. In many cases it may be at least 7 or even at least 8.5 or 9 dl/g, and often at least 10 dl/g and more preferably at least 12 dl/g and particularly at least 14 or 15 dl/g. There is no maximum molecular weight necessary for the this cationic polymer of charge density below 3 mEq per gram and so there is no particular upper value of intrinsic viscosity. In fact the intrinsic viscosity may even be as high as 30 dl/g or higher. Generally though the first polymeric retention aid often has an intrinsic viscosity of up to 25 dl/g, for instance up to 20 dl/g.

Intrinsic viscosity of polymers may be determined by preparing an aqueous solution of the polymer (0.5-1% w/w) based on the active content of the polymer. 2 g of this 0.5-1% polymer solution is diluted to 100 ml in a volumetric flask with 50 ml of 2M sodium chloride solution that is buffered to pH 7.0 (using 1.56 g sodium dihydrogen phosphate and 32.26 g disodium hydrogen phosphate per litre of deionised water) and the whole is diluted to the 100 ml mark with deionised water. The intrinsic viscosity of the polymers is measured using a Number 1 suspended level viscometer at 25°C. in 1M buffered salt solution. Intrinsic viscosity values stated are determined according to this method unless otherwise stated.

Desirably the polymers of either or both of the first and/or second polymeric retention aids may be provided as reverse-phase emulsions prepared by reverse phase emulsion polymerisation, optionally followed by dehydration under reduced pressure and temperature and often referred to as azeotropic dehydration to form a dispersion of polymer particles in oil. Alternatively the polymer may be provided in the form of beads and prepared by reverse phase suspension polymerisation, or prepared as a powder by aqueous solution polymerisation followed by comminution, drying and then grinding. The polymers may be produced as beads by suspension polymerisation or as a water-in-oil emulsion or dispersion by water-in-oil emulsion polymerisation, for example according to a process defined by EP-A-150933, EP-A-102760 or EP-A126528.

Generally the two different cationic polymers that form the cationic polymer blend may be each made into aqueous solutions separately before being combined. Alternatively, it may be desirable in some instances to make the polymer blend by dissolving the two different cationic polymers together. Typically aqueous solutions of the two polymeric retention aids may be achieved by individually dissolving the respective polymers into water. This may for instance be achieved in a suitable polymer solution make up device. Such equipment is described in the prior art and for instance commercialized by BASF under the trademark Jet Wet™.

One convenient way of preparing the blend is by flowing one of the cationic polymers into a feed line carrying the other cationic polymer form a blend of the two polymers which is then delivered into the cellulosic thin stock suspension. Alternatively, it may be desirable to combine the

two polymers and then to store the blend in a storage vessel, for subsequent delivery to the thin stock suspension.

The blend of cationic polymers, which is generally present as an aqueous blend, may contain the cationic polymer (a) having a charge density of from 0.5 to below 3 mEq per gram and a molar mass of greater than 700,000 Da at a concentration of at least 0.05% and often up to 10% or 20% or 30% or more, for instance at least 1% or at least 2% (based on total weight of blend) and the cationic polymer (b) with a charge density of below 3 mEq per gram and an intrinsic viscosity of at least 4 dl/g at a concentration of at least 0.05%, at least 0.1% or at least 0.2% and often up to 1% or 2%, although in some cases it may be desirable for the concentration to be as much as 5% (based on total weight of blend). The exact ratio of the two different cationic polymers will depend upon the desired dosage required for each respective cationic polymer. Generally the dose of cationic polymer (a) of charge density of from 0.5 to below 3 mEq per gram and molar mass of at least 700,000 may be at least 50 ppm and often at least 100 ppm. Frequently the dose will be at least 200 ppm and in some cases at least 500 ppm. The dose may be as high as 3000 ppm or higher but often will be up to 2500 ppm and in some cases up to 2000 ppm.

Usually the dose of cationic polymer (b) of charge density below 3 mEq per gram and intrinsic viscosity at least 4 dl/g may be at least 50 ppm and frequently at least 100 ppm. Typical doses may be up to 1000 ppm although doses in the range of at least 150 ppm or at least 200 ppm up to a dose of 600 ppm may often be particularly suitable. All dosages 30 of the respective cationic polymers based on the active weight of cationic polymer on the dry weight of cellulosic thin stock suspension.

The microparticulate material employed in the present invention may be any suitable finely divided particulate material. Suitably it may be selected from the group consisting of silica based particles, silica microgels, colloidal silica, silica sols, silica gels, polysilicates, cationic silica, aluminosilicates, polyaluminosilicates, borosilicates, polyborosilicates, zeolites, bentonite, hectorite, smectites, montmorillonites, nontronites, saponite, saucinite, hormites, attapulgites, sepiolites, anionic cross-linked polymeric microparticles of particle size below 750 nm and nanocellulose.

The silica may be for example any colloidal silica, for instance as described in WO-A-8600100. The polysilicate may be a colloidal silicic acid as described in U.S. Pat. No. 4,388,150. Polysilicates may be prepared by acidifying an aqueous solution of an alkali metal silicate. The polyaluminosilicates may be for instance aluminated polysilicic acid, made by first forming polysilicic acid microparticles and then post treating with aluminium salts, for instance as described in U.S. Pat. No. 5,176,891. Such polyaluminosilicates consist of silicic microparticles with the aluminium located preferentially at the surface.

Alternatively the polyaluminosilicates may be polyparticulate polysilicic microgels of surface area in excess of 1000 m<sup>2</sup>/g formed by reacting an alkali metal silicate with acid and water soluble aluminium salts, for instance as described in U.S. Pat. No. 5,482,693. Typically the polyaluminosilicates may have a mole ratio of alumina:silica of between 1:10 and 1:1500.

The siliceous material may be a colloidal borosilicate, for instance as described in WO-A9916708.

The swellable clays may for instance be typically a bentonite type clay. The preferred clays are swellable in water and include clays which are naturally water swellable or clays which can be modified, for instance by ion exchange

to render them water swellable. Suitable water swellable clays include but are not limited to clays often referred to as hectorite, smectites, montmorillonites, nontronites, saponite, saucnite, hormites, attapulgites and sepiolites. Typical anionic swelling clays are described in EP-A-235893 and EP-A-335575.

Most preferably the clay is a bentonite type clay. The bentonite may be provided as an alkali metal bentonite. Bentonites occur naturally either as alkaline bentonites, such as sodium bentonite or as the alkaline earth metal salt, usually the calcium or magnesium salt. Generally the alkaline earth metal bentonites are activated by treatment with sodium carbonate or sodium bicarbonate. Activated swellable bentonite clay is often supplied to the paper mill as dry powder.

Alternatively the bentonite may be provided as a high solids flowable slurry, for example at least 15 or 20% solids, for instance as described in EP-A-485124, WO-A-9733040 and WO-A-9733041.

The cross-linked polymeric microparticles may be made as microemulsions by a process employing an aqueous solution comprising a cationic or anionic monomer and crosslinking agent; an oil comprising a saturated hydrocarbon; and an effective amount of a surfactant sufficient to produce particles of less than about 0.75 micron in unswollen number average particle size diameter. Microbeads are also made as microgels by procedures described by Ying Huang et. al., *Makromol. Chem.* 186, 273-281 (1985) or may be obtained commercially as microlatices. The term "microparticle", as used herein, is meant to include all of these configurations, i.e. microbeads per se, microgels and microlatices.

The polymeric microparticles of this invention are preferably prepared by polymerization of the monomers in an emulsion as disclosed in application, EP-484617. Polymerization in microemulsions and inverse emulsions may be used as is known to those skilled in this art.

The cellulosic suspension used for making the pulp in the present invention may be made by conventional methods, for instance from wood or other feedstock. Deinked waste paper or board may be used to provide some of it. For instance the wood may be debarked and then subjected to grinding, chemical or heat pulping techniques, for instance to make a mechanical pulp, a thermomechanical pulp or a chemical pulp. The fibre may be bleached, for instance by using a conventional bleaching process, such as employing magnesium bisulphite or hydrosulphite. The pulp may have been washed and drained and rewashed with water or other aqueous wash liquor prior to reaching the final drainage stage on the pulp making machine.

The cellulosic thin stock suspension may contain mechanical fibre. By mechanical fibre we mean that the cellulosic suspension comprises mechanical pulp, indicating any wood pulp manufactured wholly or in part by a mechanical process, including stone ground wood (SGW), pressurised ground wood (PGW), thermomechanical pulp (TMP), chemithermomechanical pulp (CTMP) or bleached chemithermomechanical pulp (BCTMP). Mechanical paper grades contain different amounts of mechanical pulp, which is usually included in order to provide the desired optical and mechanical properties. In some cases the pulp used in making the filled paper may be formed of entirely of one or more of the aforementioned mechanical pulps. In addition to mechanical pulps other pulps are often included in the cellulosic suspension. Typically the other pulps may form at least 10% by weight of the total fibre content. These other

pulps the included in the paper recipe include deinked pulp and sulphate pulp (often referred to as kraft pulp).

The following examples illustrate the invention.

## EXAMPLES

### Example 1

#### Confidential Trial in a Paper Manufacturing Process

The mill produces woodfree coated paper on a gap former. The furnish is a 100% bleached chemical pulp consisting of 25% birch and 75% pine. The Canadian Standard Freeness of birch (short fibre) is 350-450 and the pine (long fibre) is 500-560. The fresh filler is PCC (precipitated calcium carbonate) and was included in the stock in an amount of 10%. The PCC were produced on site having an average particle size of 2.3  $\mu\text{m}$ . The consistency of the stock at the headbox is 0.8%.

Machine speed and retention levels depends on basis weight—the higher basis weights (above 75 gsm) run at lower speeds due to a steam (dryer) limitation but with higher retention values. The retention aid in use is the Hydrocol system with Polymin 1830 as the PAM (cationic polyacrylamide containing 10 mol percent cationic monomer units) added pre-screen and the bentonite added post screen. Bentonite is added with typical dosage rates of 2.4 kg/t (based on dry bentonite on dry furnish). Polymin 1830 having, intrinsic viscosity greater than 3 dl/g and charge density less than 3 mEq per gram, is added with a typical dosage rates of 0.2-0.4 kg/t (based on dry polymer on dry furnish). These addition rates vary depending on furnish conditions and paper properties. If higher amounts of Polymin 1830 had been applied in a conventional way deleterious effects in both sheet formation and strength properties would have been evident.

In accordance with the invention the aforementioned test is repeated with the extra addition of 0.75 kg/t (based on dry polymer on dry furnish) of Polymin VZ (polyvinylamine with a charge density greater than 0.5 mEq per gram but lower than 3 mEq per g and a molar mass of greater than 700,000 Da) into the final dilution water of the aforementioned cationic polyacrylamide to form a cationic polymer blend (Polymix) according to the present invention the moisture from the press section was reduced by 0.7% and steam consumption was reduced. The aforementioned cationic polymer blend also increased total/ash retention with a 25% lower addition of the cationic polyacrylamide with the same formation and strength values. These results were obtained on basis weights above 75 gsm of final coated paper.

The invention claimed is:

1. A process of making paper or paperboard, comprising subjecting a cellulosic thin stock to one or more shear stages and then draining through a moving screen to form a sheet which is dried,

wherein the process employs a retention system which is applied to the thin stock, the retention system comprising as components

- a blend of different cationic polymers, and
- a microparticulate material, which microparticulate material is selected from colloidal silica and bentonite, in which the blend of cationic polymers comprises:
  - from 50 ppm to 3000 ppm dose rate of a cationic polymer having a charge density of from 1 to 2 mEq per gram and a molar mass of from greater than 700,000 Da

**11**

- to 3 million Da, which cationic polymer is selected from polymers comprising vinyl amine units, and
- b) from 50 ppm to 1000 ppm dose rate of a cationic polymer having a charge density of below 3 mEq per grain and an intrinsic viscosity of at least 10 dl/g, which cationic polymer is a cationic polyacrylamide comprising acrylamide and from 5 to 10 mole % of at least one water-soluble cationic ethylenically unsaturated monomer,
- wherein i) the blend of cationic polymers is dosed into the thin stock prior to the final shearing stage and ii) the microparticulate material is dosed into the thin stock after the final shearing stage, and
- wherein the ppm dose rate is based on the active weight of the cationic polymer relative to a dry weight of the cellulosic thin stock suspension,
- wherein one of the components of the retention system is dosed into the thin stock after the final shearing stage and the other is dosed into the thin stock before the final shearing stage.
2. The process according to claim 1, wherein a) the cationic polymer having a charge density of from 1 to 2 mEq

**12**

per gram and molar mass of from greater than 700,000 Da to 3 million Da comprises polyvinylamine and partially hydrolysed polyvinyl carboxamides.

3. The process according to claim 1, wherein b) the at least one water-soluble cationic ethylenically unsaturated monomer is selected from the group consisting of quaternary or acid salts of &alkyl amino alkyl (meth) acrylates, quaternary or acid salts of dalkyl amino alkyl (meth) acylamides and dialkyl diallyl ammonium halides.

10 4. The process according to claim 1, wherein the molar mass of the cationic polymer a) is from 1.5 to 2.5 million Da.

5 5. The process according to claim 1, wherein b) the at least one water-soluble cationic ethylenically unsaturated monomer of the cationic polyacrylamide is a methyl chloride quaternary ammonium salt of dimethylamino ethyl acrylate.

15 6. The process according to claim 1, wherein a dose amount of the cationic polymer b) is from 50 ppm to 600 ppm, wherein the dose amount is based on the active weight of the cationic polymer relative to the dry weight of the cellulosic thin stock suspension.

\* \* \* \* \*